

## UNITED STATES PATENT OFFICE

ERNEST LECOCQ, OF BRUSSELS, BELGIUM

## PROCESS FOR SIZING PAPER

No Drawing. Application filed May 13, 1928, Serial No. 362,853, and in Belgium June 8, 1928.

The present invention relates to a process for sizing paper, particularly to sizing with resin.

In the processes of this type at present in use, the bodies generally added in the beating engine are composed of mineral and agglutinant resin soaps. Resin is for example converted into resin soap by an alkali such as sodium carbonate or sodium hydroxide.

10 These resin soaps (sizing milk) dissolve in the water and penetrate the fibres of the paper pulp contained in the beater. The resin is then precipitated on the fibres of the pulp by means of an aluminium salt. An 15 alum or sulphate or aluminium which decomposes the alkaline resinate or the resin soap is generally used. This decomposition takes place in an acid medium.

20 The disadvantages of the majority of these processes are their high cost, the presence of impurities and the fouling of the metal gauze owing to the low solubility of the materials.

25 The object of the present invention is to remove these disadvantages and to facilitate resin sizing and colouring of the paper, using a product of low value.

According to the invention, a bi-sulphate of an alkaline metal is used for this purpose either alone with the agglutinant, or mixed 30 with other mineral and vegetable substances, particularly aluminium sulphate.

A process carried out according to the invention is described below by way of example. 40 gms. of alkaline resinate obtained by 35 the action of an alkaline salt on resin are dissolved in one litre of hot water and the solution is poured into the beater containing 200 kgs. of the paper pulp to be sized. A second preparation is obtained by dissolving 180 40 gms. of aluminium sulphate and 200 gms. of sodium bi-sulphate in water, the mixture being poured into the beater already containing the resinate. The solutions of sodium bi-sulphate and aluminium sulphate are preferably added separately. The solution of bi-sulphate is poured into the beater some time (if possible half an hour) after the resinate and the solution of aluminium sulphate some time after the bi-sulphate (if possible a quarter of an hour). The bi-sulphate solution is

preferably added before the aluminium sulphate in a tank containing the paper pulp. If the resultant sizing is insufficient, aluminium sulphate is preferably added. The acidity of the pulp can then be wholly or partially neutralized in any known manner by means of a base or calcium carbonate. About 1 kg. of powdered chalk is preferably used for each kg. of sulphuric acid (66° Bé.) to be neutralized. The charge is completed in order to give the desired percentage by adding an inert substance such as kaolin.

A paper of better quality than by any other process is obtained, the retail price of which is five or six times less. It is to be noted that the acid sulphates of the alkaline metals are obtained in a purer form than aluminium sulphate. They are more easily freed from iron and are better mordants for fixing dyes, etc.

This process using alkaline bi-sulphate alone is used for ordinary papers and papers comprising old sized papers. The combined process using aluminium sulphate is applicable to all kinds of paper but for complete 75 sizing (strong size) it is preferable to use a third of aluminium sulphate, 1 kg. of sodium bi-sulphate replacing 2.5 kgs. of aluminium sulphate.

It is obvious that the constituents can be varied but one of the solutions used for the sizing must always, according to the invention, contain a sulphate or bi-sulphate of an alkaline metal.

The relative proportions of each of the constituents are not fixed and can be varied according to the desires of individual customers and according to the price to be paid.

What I claim is:

1. In a process for sizing paper by means of an agglutinant constituting a resin soap, treating said resin soap and the paper pulp with bisulfate of an alkaline metal.

2. In a process for sizing paper by means of an agglutinant constituting a resin soap, treating said resin soap and the paper pulps with bisulphate of an alkaline metal used in the form of a solution of sodium bisulphate.

3. In a process for sizing paper by means of an agglutinant constituting a resin soap,

treating said resin soap and the paper pulp with a solution of a bisulphate of an alkaline metal and a solution of aluminium sulphate.

4. In a process for sizing paper by means of an agglutinant constituting a resin soap, treating said resin soap and the paper pulp with a solution of bisulphate of an alkaline metal and treating the mixture afterwards with a solution of aluminium sulphate.

10 5. In a process for sizing paper by means of an agglutinant constituting a resin soap, mixing a solution of a bisulphate of an alkaline metal with a solution of aluminium sulphate and treating the resin soap and paper pulp with the said mixture.

15 6. In a process for sizing paper by means of an agglutinant constituting a resin soap, treating said resin soap and the paper pulp with a solution of approximately three parts of sodium bisulphate and a solution of two parts of aluminium sulphate.

20 7. In a process for sizing paper by means of an agglutinant constituting a resin soap, treating said resin soap and the paper pulp with bisulphate of an alkaline metal, and neutralizing the acidity of the paper pulp by a base.

25 8. In a process for sizing paper by means of an agglutinant constituting a resin soap, treating said resin soap and the paper pulp with bisulphate of an alkaline metal and neutralizing the acidity of the paper pulp by calcium carbonate.

30 9. In a process for sizing paper by means of an agglutinant constituting a resin soap, treating said resin soap and the paper pulp with bisulphate of an alkaline metal and neutralizing the acidity of the paper pulp by powdered chalk.

35 40 In testimony whereof I have affixed my signature,

ERNEST LECOCQ.

45

50

55

60

65